

May 4, 1954

H. R. MONTGOMERY ET AL  
PROCESS OF COATING CARBONACEOUS  
MATERIAL WITH SILICON CARBIDE  
Filed Oct. 26, 1951

2,677,627



Inventors  
HAROLD R. MONTGOMERY  
JAN WALTER SZYMASZEK

By *George L. Compton*  
Attorney

## UNITED STATES PATENT OFFICE

2,677,627

## PROCESS OF COATING CARBONACEOUS MATERIAL WITH SILICON CARBIDE

Harold R. Montgomery and Jan Walter Szymaszek, Niagara Falls, Ontario, Canada, assignors to Norton Company, Worcester, Mass., a corporation of Massachusetts

Application October 26, 1951, Serial No. 253,302

10 Claims. (Cl. 117—106)

1

The invention relates to a process for coating carbonaceous material such as graphite with silicon carbide.

One object of the invention is to produce superior exhaust nozzles for guided missiles. Another object is to produce superior rocket nozzles. Another object is to produce superior combustion chambers. Another object is to produce superior crucibles.

Another object of the invention is to provide a process for forming silicon carbide in situ on graphite or other carbonaceous pieces with simple equipment. Another object is to provide a process for coating articles with silicon carbide which produces heavy and strongly adherent coatings. Another object of the invention is to provide a thoroughly practical process for the manufacture of Venturi tubes and the like.

Other objects will be in part obvious or in part pointed out hereinafter. In the drawing the single figure is a vertical axial sectional view of inner and outer crucibles, an induction coil and of Venturi nozzles made of graphite being coated with silicon carbide.

For guided missiles, rockets and the like Venturi nozzles and combustion chambers capable of withstanding great heat are needed. However they do not have to have a long life. We have discovered a process for making superior nozzles with Venturi bores that will withstand intense heat for a long enough time to be quite successful for use in such guided missiles and rockets.

We start with pieces of graphite because graphite can readily be machined. For example the shapes 1 are made from solid cylinders of graphite by boring them and then shaping the bores in a turret lathe using shaped tools. These shaped tools are made of soft steel and this greatly simplifies the problem of making the tools to the exact shape desired; a problem which would be difficult using hard tool material because the Venturi shape is not simple. Two tools are used for shaping the bores, one for each end, and each tool cuts on each side thereof thus to balance the cutting forces and then a third tool is used to finish the smallest diameter of the bore at the limit of machining by the other tools to make a bore smooth from end to end without any tool marks and of perfect Venturi shape.

The shapes 1 which are to be nozzles are set on graphite bars 2 which are preferably triangular in cross section and are supported by a circular graphite plate 3 resting on graphite bars 4, which can be square or rectangular in cross section, the bars 4 being placed across the open

2

top of an inner graphite crucible 5 filled almost full with silica sand 6. The graphite crucible 5 rests on graphite blocks 7 on the bottom of an outer graphite crucible 8 having a graphite cover 9.

Through the cover 9, conveniently in the center thereof, is a bore 10. In a counterbore of the bore 10 is a graphite tube 11 which acts as a chimney. Extending into a dead end bore into the cover at an angle to the vertical is a graphite tube 12 with two bores 13 and 14 and a cut-out 15 at the inner end; this is a pyrometer tube and the reason for having two bores and a cut-out is to blow gas, such as nitrogen, through it from the outer end to get rid of fumes which would obscure the dead end of the bore in the cover 8 the color of which is matched to the hot wire of the pyrometer in order to determine the temperature of the apparatus.

20 Outside of the crucible 8 is coiled copper tubing 16 through which water is flowing and through the metal of which an alternating current of electricity at high frequency is flowing. The coiled copper tubing 16 is the primary of high frequency induction apparatus; the secondary is the crucible 8 and the cover 9. Inside of the coil 16 is a sheet of asbestos 17 coiled into a cylinder and inside of the asbestos sheet 17 and under the crucible and over the cover 9 is 30 comminuted zirconia 18 which is very heavy and is a good insulator of heat and, where cool as on the outside, a non-conductor of electricity. The bottom of the coil 16 and the lower layer of zirconia rest upon fire clay bricks 19.

35 The process may now best be described by giving an illustrative example.

*Example 1*

For coating certain nozzles and cylinders with silicon carbide the apparatus described was used 40 the crucible 8 having been thirty inches in diameter and the other dimensions of the crucible 8 and of the other parts of the apparatus having been in proportion about as shown in the drawing. The nozzles in this case were 3 1/4 inches 45 long and 2 1/8 inches in diameter with Venturi bores about the same shape as in the shapes 1; but these nozzles were smaller in proportion to the apparatus and there were thirteen of them. The apparatus having been assembled with the nozzles on bars 2, the induction machine (not shown) was started and delivered electric current at a frequency of 1000 cycles a second with a power of 240 kilowatts to the coil 16. The 50 electromotive force was 365 volts. This input

was maintained for two hours and twenty minutes whereupon the E. M. F. was dropped to 285 volts and the power to 170 kw. and this input was maintained for one hour more and then the current was turned off completely and the apparatus was allowed to cool. The nozzles were found to be coated with silicon carbide inside and outside to a depth of about .020" to .030". The temperature inside of the crucible 5 for the last hour was approximately 2350° C.

The process is believed to work as follows: The silica sand 6 melts at about 1700° C. and boils at 2230° C. Therefore when the crucible 5 reached about 2240° C. the liquid silica boiled violently. At first the gases passed off through the chimney 11 but later that became plugged with condensed silica and then an appreciable pressure built up within the crucible 8; sometimes the cover 9 with the heavy zirconia 13 thereon has been lifted and when that happened the power was cut down for a while. In the particular run described in Example I, however, the cover 9 did not rise.

The silica vapor in the crucible 8 on striking the pieces 1 reacts with the graphite (carbon) to form silicon carbide which is thus integral with the pieces 1. Of course the inside of the crucible 8 and the under side of the cover 9 are also coated with silicon carbide but that is not a detriment. The first time the apparatus is used a large amount of silica sand is used up coating the inside of the crucible 8; thereafter less silica sand is used up because the coating process proceeds more slowly after the initial stages as the graphite does not have such ready access to the silica vapor. But the silicon carbide layer is somewhat porous so the reaction



continues although at a gradually decreasing rate. When the apparatus has been used a number of times the crucible 8 is found to be lined with silicon carbide inside and also the bottom of the cover 9 has a coating of silicon carbide and the coating and lining of the pieces 1 takes less time than in the first operation. The operation described in Example I was done with apparatus which had been used before. As an incident of the process the plate 3 and also the crucible 5, the bars 2 and 4 and the blocks 7 are likewise coated with silicon carbide.

Our process is much more effective than the process of coating graphite and the like by heating it in the presence of silicon. Silicon carbide dissociates at 2500° C. so therefore in any process for coating anything with silicon carbide the temperature has to be kept below that figure, but silicon does not boil until it reaches 2600° C. so the process of coating graphite with silicon carbide by heating it in the presence of silicon is dependent upon the presence of a minor proportion of silicon vapor in the atmosphere and the process is slow and it is difficult to form a thick coating using the silicon process. But in our process the atmosphere in the crucible 8 is heavily charged with silica vapor  $\text{SiO}_2$ , the coating of silicon carbide is relatively quickly formed and thick strong coatings can be made.

The reason why we use a plate 3 to cover the crucible 5 instead of laying the bars 2 across an open top crucible 5 with the pieces 1 on the bars 2 is that when the silica boils a blast of vapor is formed which will corrode the pieces 1, that is to say eat them away whenever the vapor impinges thereon. In other words the plate 3

is a baffle to break up the flow and to cause turbulence and to shield the pieces 1 from a fast moving stream of gaseous silica. At all events the setup illustrated is effective while removal of the plate 3 frequently spoils the pieces 1. The baffle plate 3 thus cuts down the velocity of the silica gas and any other arrangement to cut down the velocity of the gas at the locus of the pieces 1 could be used. This feature may be referred to as protecting the pieces from direct impact of the silica gas. We will now give another example of the process of the invention.

#### Example II

15 Using a graphite crucible 8 of the same size as already described and other parts in proportion about as shown in the drawing we coated twelve graphite pieces to form nozzles. The pieces were  $3\frac{1}{4}$  inches long and  $2\frac{1}{8}$  inches in diameter and the bores had about the same Venturi shape as the bores in the pieces 1 in the drawing. For one hour and a half the coil 16 was energized with electric current at 315 volts, 230 kilowatts and a frequency of 1000 cycles per second, then for one hour at 315 volts, 240 kilowatts and the same frequency, then for one hour at 285 volts, 170 kilowatts and the same frequency. The apparatus had been used before so the inside of the crucible 8 and the under side of the cover 9 and the crucible 5 and plate 3 were coated with silicon carbide. The temperature of 2350° C. was reached and held for the last hour. The pieces were well coated, the coating was about .020" to .030" thick and absolutely integral with the underlying graphite. The outside diameter grew only .004" to .006" (.002" to .003" on the radius) showing that a good deal of the graphite was converted to silicon carbide. (The Venturi bore was coated with silicon carbide .020" to .030" thick and was everywhere reduced in diameter by .004" to .006".) Thus it is not a case of merely forming a coating on a piece of graphite, an outer layer and also an inner layer of graphite is converted to silicon carbide while more silicon carbide forms thereover. The same result was also achieved in Example I.

#### Example III

20 Using similar apparatus as in Examples I and II with an old crucible 8 well coated with silicon carbide on the inside and an old cover 9 well coated with silicon carbide on the under side but with a new plate 3 and crucible 5 (the blocks 7 were omitted in this run in order to leave enough space for the pieces) the coil 16 was energized at 320 volts, 220 kilowatts, 1000 cycles to coat four graphite pieces to make nozzles, 8 inches in diameter, 12 inches long with Venturi bores, and to coat four hollow cylinders to make chambers, 8 inches outside diameter,  $7\frac{1}{2}$  inches inside diameter and 10 inches long. The above input was maintained for one hour then the load increased to 240 kilowatts, voltage same. This input was maintained for another hour whereupon, with the same voltage the load increased to 250 kilowatts. At this time, namely at the end of two hours, the chimney 11 was found to be plugged. After another half hour the voltage was dropped to 260 and the load became 170 kilowatts. The temperature had now reached about 2350° C. The latter input, 260 volts, 170 kilowatts was maintained for another hour holding the temperature inside the crucible 8 at 2350° C. or thereabouts. Then the current was cut off and

the apparatus was allowed to cool. The pieces were found to be coated everywhere by a coating .020" to .030" deep but had grown (outside and inside) only .002" to .003" on the radius. Of course this growth makes the bore smaller by the amount stated.

The chimney 11 (which was 24 inches high) took on a coating of silicon carbide in its bore adjacent the lower end but frequently became plugged with silica about half way up. There was always some plugging of the chimney with silica but this plugging did not in every run completely block the chimney although in many runs it did. This plugging with silica rather conclusively shows that the atmosphere in the 10 crucible was silica and not silicon. However we believe that the silica in vapor phase may have included some silicon monoxide,  $\text{SiO}$ , as well as the vapor phase silicon dioxide,  $\text{SiO}_2$ . The oxygen lost would combine with carbon to form carbon monoxide. All air originally in the crucible 8 had been driven out of the chimney 11 long before the plugging occurred. The same chimney tube 11 was, however, used over and over again 15 since the silica plugging it was removed with no great difficulty with iron rods.

The Venturi bore may, in some cases, be a bore comprising a pair of frusto-cones on a single axis with the small ends towards each other but more often the bore is a non-symmetrical negative hyperboloid. An hyperboloid is a volume defined by rotating an hyperbola around an axis. The hyperboloid is negative when its surface is concavo-convex. The bore is non-symmetrical when one mouth is larger than the other one. If the pieces are made of amorphous carbon hard cutting tools are required. Such tools are more difficult to shape to curves such as hyperbolas and therefore it is an advantage to cut the pieces 20 out of graphite which can be cut with soft steel since the soft steel tools can be more easily shaped. The cutting tools are usually made to approximate shape in a lathe and then finished by hand to accurate hyperbola shape using files and abrasive cloth.

A great advantage of our process is that there is so little growth (and what growth there is is evenly distributed) so nozzles can be made within tolerances of plus or minus one thousandth of an inch everywhere. Allowance is, of course, 25 made for such growth as is obtained.

For the manufacture of very large nozzles the process of the invention can also be used for coating sectors of cylindrical pieces with Venturi bores so that when the sectors are assembled a complete nozzle will be formed. In one case the shape consisted of twenty sectors which were coated with silicon carbide and eventually assembled in a steel shell with refractory cement.

Within the limits of this invention any carbonaceous material can be coated which will remain in the solid phase at  $2230^\circ \text{C}$ . This includes amorphous carbon and graphite and pieces of other material mixed therewith. The range of top temperatures for carrying out this invention is from the boiling point of silica (which we believe is close to  $2230^\circ \text{C}$ ) to the incipient decomposition of silicon carbide (we believe it starts to decompose at about  $2450^\circ \text{C}$ . although decomposition is not rapid until about  $2500^\circ \text{C}$ ). Furthermore at above  $2450^\circ \text{C}$ . the boiling of the silica appears to be too violent for the best results. The temperature should be maintained between these limits for at least one half hour to produce an adequate coating.

We have found it is really immaterial whether the chimney 11 becomes plugged or not and in any event the pressure in the crucible 8 never rises much above one pound per square inch gauge pressure and frequently is at atmospheric pressure.

Graphite has great thermal shock resistance and can be easily machined into desired shapes. However it oxidizes readily at high temperatures. 10 Silicon carbide is very refractory and not easily oxidized even at the temperatures of the jets in rockets and other missiles. It is resistant to the erosive effect of the jets, the gases of which sometimes reach a velocity of 4000 feet per second, 15 while graphite is not resistant to such erosive effect. And silicon carbide is difficult to shape and almost impossible to machine. Hence by coating graphite with silicon carbide, we utilize the good properties of each material without detriment from the bad properties of either.

Features of the invention are that the pieces to be coated are spaced from the comminuted silica (silica sand) and are not buried in anything, i. e. they are surrounded by air in the 20 first place and during the process they are surrounded by gaseous silica with some carbon monoxide mixed therewith instead of being buried in the sand. Another feature is that the heating is done by electric induction which makes possible excellent control without which control the results are sporadic and uncertain. Furthermore, induction heating makes possible uniform heating which is highly desirable.

It will thus be seen that there has been provided by this invention a process for coating carbonaceous material (especially graphite) with silicon carbide in accordance with which the various objects hereinbefore set forth together with many thoroughly practical advantages are 30 successfully achieved. As many possible embodiments might be made of the mechanical features of the above invention and as many changes might be made in the embodiments above set forth it is to be understood that all matter hereinbefore set forth or shown in the drawing is to 35 be interpreted as illustrative and not in a limiting sense.

We claim:

1. Process of coating a carbon body with silicon carbide comprising placing said carbon body in a closed carbon container containing comminuted silica spaced from said body, heating the container to the boiling point of the silica while protecting the body from direct impact of the gaseous silica formed and keeping the temperature below the temperature of incipient decomposition of silicon carbide and maintaining the temperature of the container between the boiling point of silica and the temperature of incipient decomposition 40 of silicon carbide for at least one half hour, the coating being formed by the reaction of silica gas with the carbon material.

2. Process according to claim 1 in which the body is a body of graphite.

3. Process according to claim 2 in which the container is made of graphite.

4. Process according to claim 1 in which the container is made of graphite.

5. Process for the manufacture of articles 50 coated with silicon carbide comprising machining a piece of graphite to the required shape, placing it in a closed carbon container with a quantity of comminuted silica therein but spaced from the comminuted silica, heating the container to the 55 boiling point of the silica while protecting the 75

piece from direct impact of the gaseous silica formed and keeping the temperature below the temperature of incipient decomposition of silicon carbide and maintaining the temperature of the container between the boiling point of silica and the temperature of incipient decomposition of silicon carbide for at least one half hour, the coating being formed by the reaction of silica gas with the graphite.

6. Process according to claim 5 in which the container is made of graphite.

7. Process according to claim 1 in which the heating is done by electric induction whereby to secure substantially uniform heating of the silica and of the carbon body.

8. Process according to claim 7 in which the carbon body is a body of graphite.

9. Process according to claim 8 in which the container is made of graphite.

10. Process according to claim 1 in which the heating is done by electric induction whereby to secure substantially uniform heating of the silica and of the carbon body and in which the container is made of graphite.

References Cited in the file of this patent

UNITED STATES PATENTS

| Number    | Name          | Date          |
|-----------|---------------|---------------|
| 1,658,647 | Miller        | Feb. 7, 1928  |
| 2,431,326 | Heyroth       | Nov. 25, 1947 |
| 2,439,983 | Morgan et al. | Apr. 20, 1948 |
| 2,463,791 | Morgan        | Mar. 8, 1949  |